

March 30, 1937.

R. H. VARIAN

2,075,377

MEANS AND METHOD OF FORMING DISCRETE AREAS

Filed March 13, 1935.

Fig. 2.



Fig. 3.



Fig. 1.



Fig. 4.



INVENTOR,  
RUSSELL H. VARIAN.  
BY *Dippincott & Metcalf*  
ATTORNEYS.

## UNITED STATES PATENT OFFICE

2,075,377

MEANS AND METHOD OF FORMING DIS-  
CRETE AREASRussell H. Varian, San Francisco, Calif., assignor  
to Farnsworth Television Incorporated, a cor-  
poration of California

Application March 13, 1935, Serial No. 10,883

5 Claims. (Cl. 250—27.5)

My invention relates to a means and method of forming discrete conductive areas, and more particularly to a means and method of forming a mosaic photoelectric surface.

- 5 Among the objects of my invention are: to provide a means and method for forming a surface having a plurality of discrete, closely adjacent conductive islands; to provide a mosaic photoelectric emitter; to provide a mosaic surface 10 having a plurality of discrete conductive areas upon which photoelectric material may be deposited; to provide a means and method for preparing a silver surface for the deposition of photoelectric material thereon; to provide a means and 15 method of condensing a vaporizable material as a discontinuous surface; and to provide a means and method for regulating the sensitivity of a photoemissive substance during the activation thereof when deposited in discrete areas.
- 20 Other objects of my invention will be apparent or will be specifically pointed out in the description forming a part of this specification, but I do not limit myself to the embodiment of the invention herein described, as various forms may 25 be adopted within the scope of the claims.

Referring to the figures which illustrate several steps in the formation of a preferred photoelectric cathode:

Figure 1 is a plan view of a preferred type of 30 photoelectric cathode, showing the distribution of the treated surfaces thereof.

Figure 2 illustrates a step in the formation of a mosaic silver surface upon a preferred form of cathode.

35 Figure 3 is a longitudinal sectional view of a television dissector tube similar to that described in the application of Philo T. Farnsworth, Serial No. 668,066, filed April 26, 1933, for an Image dissector, wherein the mosaic photoelectric cathode 40 of my invention is mounted.

Figure 4 is a sectional view through a photoelectric cathode, on which a mosaic photoelectric layer has been formed on a loosely deposited, finely divided, insulating powder.

45 In many instances, one example of which is the cathode of the dissector tube disclosed in the above identified application, it is desirable to make a photoelectric emitter comprising a plurality of closely adjacent discrete emitting 50 islands. A number of methods are known in the art whereby such mosaic emitters can be produced, one of which includes the step of evaporating silver through a fine screen onto an insulating surface. It is quite common to project the 55 silver vapor from a point source above the screen

and the surface. The silver thus deposited in a pattern determined by the screen characteristics is subsequently oxidized, caesium vapor admitted to the tube for deposit on the silver, and the caesium activated in the usual way. The particular type of mosaic emitter thus formed, however, is not ideal. The most important disadvantages of the screen method are, using a mica sheet for an example of the insulator upon which the deposit is made:

5 1. A mono-molecular layer of alkali metal on the mica surface between the islands may easily cause a leak between the islands.

10 2. The regular arrangement of the islands, when combined with a moving beam or other 15 scan arrangement of definite aperture size, can easily produce interference patterns similar to those seen when looking through two wire screens.

15 3. The spaces between the islands are neces- 20 sarily large, due to the size of the screen material, and the islands themselves are relatively large, due to the practical inability to make a screen of sufficiently fine mesh to produce the number of islands usually desired.

25 There is another method of making a mosaic surface wherein active material is evaporated directly onto an insulating surface, the identity of the islands relying on a tendency of the deposited material to group itself in minute balls on the 30 surface. This method, however, is uncertain in its action and the method is hardly applicable to commercial production, it being very difficult to form uniform distribution over relatively large areas.

35 Broadly stated, I have found that a mosaic photoelectric surface having small islands closely adjacent may be formed by evaporating a condensable metal onto a roughened and irregular surface, the indentations of which preferably 40 have overhanging edges. These edges cast shadows when the surface is exposed to metal vapor travelling in relatively straight lines from a substantially point source. I may prefer to form the conductive islands by evaporating silver onto such an indented surface, and thereafter condense alkali metal or similar photoelectric material thereon. I also prefer to oxidize the silver surface before the deposition of the photoelectric material thereon, and I have found 45 that a better emitter is eventually obtained if the oxidation is performed by oxygen ions reaching the surface by diffusion rather than with high velocities imparted thereto by excitation of the mosaic surface itself.

5

10

15

20

25

30

35

40

45

50

55

In the formation of any photoelectric surface it has hitherto been quite customary to sensitize the alkali metal, for example, by creating a glow discharge within the envelope and to check the 5 emission of the cathode during the sensitization process. With an emitter comprising a large number of discrete emitting particles, it is a complicated and difficult process to do this checking by measuring the emission of any or all of the 10 islands. I therefore prefer to provide, adjacent the mosaic surface, and preferably in the same plane therewith, an extended smooth surface upon which continuous photoelectric material is deposited. It is relatively easy to check the emission 15 from this continuous surface, and I have found when the emission from the continuous surface is at its maximum that the emission from the photoelectric islands is also at its maximum. A simple method of controlling the sensitivity of 20 the islands is thereby attained.

The roughened indented surface, having the proper overhangs, may be formed in a number of ways, as the physical characteristics only of the surface are the important factors, the particular means by which such a surface is obtained being of less consequence. I may deeply scratch and thereby roughen a relatively soft material, such as mica, to form the surface, or I may deposit upon a relatively smooth insulating surface 25 a layer of finely divided insulating powder, preferably one of such fineness that it has adherent properties. I have found that finely divided and powdered quartz is a satisfactory material to employ, but other refractory materials will be equally 30 satisfactory, the requirements for them being principally that the caesium be not able to combine with them, and that they may be deposited in such a way as to form overhangs.

Regardless, however, of how the surface is obtained, I have found that when vaporizable metals, such as silver or the alkali metals, are caused to condense upon such an indented surface, preferably from a point source, the metal atoms arriving in straight lines, that every point on the 45 roughened surface will be covered with the condensed metal which is not shaded by higher portions of the surface. The islands are insulated, one from the other, because many of the points of contact, between grains when powder is used 50 are on surfaces which are either parallel to the direction travelled by the metal ions or are under projecting portions of one or groups of grains.

Referring to the drawing for a more detailed discussion and description of my invention, I prefer to start the foundation of my cathode with a 55 surface as shown in plan in Figure 1. A mica disc 1 is preferably provided with a mask, not shown, having a square opening therein. This mask is placed over the mica sheet and powdered 60 quartz is deposited on the surface by being blown, usually in suspension, from a spray gun, for example, until a square powdered surface is deposited on the plate, as indicated by the peripheral outline 2. I then mount this mica sheet on a 65 conductive cathode plate 4, the plate being of slightly larger diameter than the mica sheet, and the sheet being held thereon by clips 5 bearing on the edge of the mica. The cathode plate with its accompanying mica sheet carrying the powder 70 layer 2, is mounted on risers 6 fastened in turn to a clamp 7, secured around a stem 9. A cathode connection lead 10 passes through the stem and connects to one of the risers. I then prefer to mount this stem in a processing envelope 11 75 and position the cathode close to one end of the

blank. On the opposite end of the blank I insert a supporting stem 12, carrying a silver chamber 14 on a chamber lead 15 sealed through the supporting stem. The chamber 14 is hollow and is provided with an aperture 16 directed toward the cathode assembly. Within this chamber I prefer to place a quantity of pure silver 17.

I then exhaust the processing envelope and heat the silver chamber, preferably by means of an eddy current coil 19 positioned outside the envelope and surrounding it, to a temperature sufficiently high to vaporize the silver 17. The vaporized metal enters the interior of the envelope, and will deposit upon both the powdered surface 2 of the mica sheet 1 and upon the clean surface. If desired, a potential may be impressed between the silver chamber and the cathode to assist the metal atoms in their traversal of the chamber. As the silver atoms are travelling from the opening 16 toward the cathode in straight lines, they arrive at the cathode in a line not greatly departing from a right angle to the plane of the cathode surface. Of course at the edges there will be a slight angle, but this angle is unimportant as long as it is not too great.

During condensation on the powder layer, shadowing will take place with a result as shown in Figure 4. The silver will be condensed upon those portions of the powder layer which present a surface normal to the oncoming silver, but will not deposit under the overhangs nor upon the sides which are parallel to the line of travel of the incoming vapor. The result is the formation of small and numerous isolated conductive silver areas on the powder layer.

It will, of course, be obvious that upon that portion of the mica surface which is not covered with powder, that silver will be deposited in a continuous layer, forming an area about the mosaic layer which is continuous and conductive. As the clips 5 of the cathode extend over onto the clean surface, the continuous silver layer will make contact thereto. The lead 10 therefore makes direct connection to the 40 continuous surface.

In experiments performed to determine the continuity of silver surfaces deposited on a clean surface and on a powdered surface, it was found that under identical conditions where the thickness of the silver deposit was the same, that the plain silver surface on the mica, without any powder had a resistance, over a given length, of three ohms. Using the same length of path for measurement, it was found that the silver which had been deposited upon powder had a resistance, in every direction, greater than  $5 \times 10^8$  ohms, thus proving that the islands are 55 completely discontinuous, allowing practically no leakage therebetween.

It will also be apparent that the size of the conductive islands, and to some extent their spacing, may be controlled by varying the size, shape, and manner of deposition. If small powder grains are deposited in a dense, relatively smooth surfaced layer, the islands will be very small and close together. If, however, the same powder is laid down in a very rough manner with large groups of grains loosely attached to each other, the islands will be relatively large. If the powder grains are made large and loosely deposited, the islands will be large and the distance between them will also be relatively large. It is therefore possible to make mosaic 60 65 70 75 80 85 90 95 100

metal layers having practically any island dimensions desired.

I have found that the mosaics formed by the means and method described above are, in their average size, well below the size of the smallest elementary scanning area desired. I have also found that they do not tend to run together into linear groups, and it is of course obvious from the way in which the islands are created that they form no pattern, being indiscriminate in their relation one to another. While I have no direct evidence that the islands have a uniform average size, I do know, when the cathode is used in a television dissector, such as will be later described, that the detail produced in the image, as reconstructed in a receiver, definitely shows, by the uniform detail, that there is no tendency for the islands to run together to form linear streams or consolidated masses which are of sufficient size to cause any blurring in the image therein.

Returning again to the cathode having a silver surface, as formed in the processing envelope 11, I next prefer to remove the silvered cathode from the processing envelope, preferably by a separation, as indicated by the dotted line 20 in Figure 2. I then prefer to mount the silvered cathode in a television dissector tube envelope 21, the glass sealing together as indicated by a ring seal 22.

The other end of the dissector tube envelope is provided with an anode assembly 24. This particular tube has been fully described in the above identified application, and as the particular form of dissector tube in which the cathode is used is no part of the instant invention, it will not be necessary to go into the function of this anode assembly in this application.

Further processing of the cathode is carried out in the tube shown in Figure 3. The tube envelope 21 is connected to a pump through a stop-cock 25, and the exhaust tube 26 is provided with a connection to a source of alkali metal vapor, preferably a bulb 27, containing caesium 29, and adapted to be heated by a gas flame or other source 30. The tube is preferably thoroughly baked and exhausted, and oxygen is admitted through the pump line into the interior of the envelope. I then prefer to form, in the neighborhood of the cathode, a ring glow discharge in the oxygen by means of the eddy current coil 19 which has been transferred to a position around the cathode end of the envelope 21. This ring discharge is maintained while oxygen ions diffuse from the discharge region into the silver surface. These oxygen ions oxidize the silver.

It will be obvious, of course, that the silver may also be oxidized directly by heat or by high frequency applied to the cathode plate behind the mica, but I have found that in every case the electrodeless ring discharge gives the best surface. Why this should be I am not at this time prepared to state, but it would appear that the oxidization by means of an oxygen ion having little or no impact velocity, gives a better surface than when heat is used or when the ions are directed into the surface with substantial impact velocity imparted by electrode potentials.

The bulb 27 is then heated to introduce caesium vapor into the envelope, where it com-

bines with the silver oxide to form a photoelectric surface on both the discrete areas and on the continuous silver area.

It is not necessary that the caesium vapor be directed onto the surface from a point source, as it appears that the caesium vapor deposits on and combines with the silver oxide without the need for direction, but does not deposit between the islands nor on the walls to any great extent.

During the deposition of the caesium, or during later activation if any additional processing is desired, the degree of sensitivity of the device may be constantly checked by illuminating the cathode, utilizing the direct connection 10 to the continuous area of the cathode for a measurement of the emission therefrom, the anode assembly being used as a collector. When the point of maximum sensitivity has been reached the exhaust tube 26 is sealed and the completed envelope removed from the exhaust system. The tube is then in the condition to be utilized as a television dissector tube, as described in the above identified application.

It will be apparent to those skilled in the art that the same means and method as above described may be utilized to form a mosaic photoelectric surface in apparatus other than that shown. Such uses will be apparent to those skilled in the art, and I do not wish to be limited by the single embodiment of the device as described in conjunction with a television dissector tube, the latter use being merely a convenient combination for purposes of illustration and description.

I claim:

1. The method of forming electrically discrete areas of a vaporizable conducting material on a surface which comprises depositing a layer of closely adjacent insulating particles on said surface, condensing said material on portions of said particles, and regulating the average size of said areas by controlling the average size of the particles deposited.

2. The method of forming discrete conductive areas which comprises forming a surface of fine insulating and refractory particles in average contact over a relatively small portion of their surface area, and projecting metal atoms thereon in substantially straight lines from a point placed above said surface.

3. The method of forming a photoelectric surface which comprises forming a layer of silver, placing said layer in oxygen, ionizing said oxygen with said silver at zero potential, and depositing a photoelectric material on the oxidized silver.

4. A photoelectric mosaic cathode comprising the following layers in order: a conducting layer, a homogeneous insulating layer, a layer of finely ground insulating powder, a layer of silver deposited in discrete areas on said powder layer, and photoelectric material deposited on said discrete areas.

5. A photoelectric mosaic cathode comprising the following layers in order: a conducting layer, a homogeneous insulating layer, a layer of adherent particles of insulating powder of heterogeneous sizes, a layer of photosensitive material deposited in discrete areas on said powder layer, said conductive layer being of at least as great an area as the area covered by the photoelectric material, and underlying said material.

RUSSELL H. VARIAN.